

# UNITED STATES PATENT OFFICE

HYMAN ELI GOLDBERG, OF CHICAGO, ILLINOIS.

## PROCESS OF METALLIZING ELECTROTYPE-MOLDS.

1,037,469.

Specification of Letters Patent.

Patented Sept. 3, 1912.

No Drawing.

Application filed August 2, 1911. Serial No. 642,032.

To all whom it may concern:

Be it known that I, HYMAN ELI GOLDBERG, a citizen of the United States, residing at Chicago, in the county of Cook and State 5 of Illinois, have invented a certain new and useful Process of Metallizing Electrotype-Molds, of which the following is a specification.

My invention relates to the process of 10 "metallizing" or preparing electrotype molds to make them conductive in order that the metal may be subsequently deposited in the ordinary manner.

It is well known that under the present 15 practice the preparation, or as it is termed in the trade, the "metallizing" of the non conductive mold involves considerable labor and inconvenience and is in several respects unsatisfactory. For example, the common 20 process of metallizing the wax mold consists of the application of fine flake graphite in dry state to said mold. This process is very objectionable because the graphite flies about in all directions to the great incon- 25 venience of the workmen. This has been overcome by the construction of special machines which brush the graphite onto the mold, but it nevertheless remains a lengthy and delicate operation. Another method 30 consists in the application of metallic powder, for instance, bronze, to the mold and then applying a solution like silver nitrate or some other metallic salt in order to cause it to "take." This process is not used much 35 in practice on account of its inconveniences. There are other processes, namely, the treatment with silver nitrate and phosphorous, and the treatment with silver nitrate and sulfureted hydrogen. These methods are 40 inconvenient and laborious and require considerable time, and frequently unless the work is very carefully done the results are imperfect and unsatisfactory.

The object of my invention is to simplify, 45 cheapen and improve the so-called process of metallizing and is accomplished in the following manner:—

I first prepare a solution of a conductive 50 solid in colloidal form in a volatile liquid, then apply this solution to the non conductive mold and finally dry the mold, thereby evaporating the solvent and causing the conductive substance to be deposited on the non conductive mold. Among the properties of 55 colloidal metals is the one that upon evaporation of their solvent they become non col-

loidal or insoluble. In my process the metal is, therefore, deposited upon the mold in a coherent, continuous, insoluble, electrically conductive layer. Among the conducting 60 solids which I employ for the preparation of the colloidal solution may be gold, silver, or graphite, et cetera, but I prefer copper. Among the solvents for the solids are water, alcohol, ether, glycerin, acetone, et cetera. 65

One method of obtaining copper and other metals in colloidal form is to form a direct current arc under water between terminals consisting of the metal to be rendered colloidal. Other methods are explained by 70 Theo. Svedberg in his published book upon the subject, entitled *Herstellung Kolloider Lösungen Anorganischer Stoffe*, 1909 edition, published by Theodore Steinkopff, Dresden, Germany. He describes methods 75 applicable to organic solvents such as alcohol, ether, glycerin and acetone and the method consists in forming an alternating current arc in the liquid and introducing the metal, for example, silver or copper, in 80 finely divided form, for example, small pieces of foil or thin sheets. The various processes are listed in the index at the end of the book, for instance, those relating to copper are listed on page 506. 85

It is the common practice to employ wax as the substance for making the electrotype mold. It will be found generally that a water colloidal solution will not wet wax readily. This objection may be avoided by 90 treating the mold previously to the application of the colloidal solution, with alcohol or similar liquid. I greatly prefer, however, to avoid the necessity for this alcohol pre-treatment by employing as the solvent one 95 which has a greater attraction for wax than water, and as such solvent I prefer ether. Another advantage in employing ether as a solvent is that whereas a colloidal solution of copper in water spoils very readily by the 100 oxidation of the copper such oxidation occurs very slowly in ether. Copper, of course, is an excellent conductor, and furthermore, copper is the metal usually employed in electrotyping and consequently by 105 employing copper for the metallizing substance I avoid mixing metals. Therefore, for all of these reasons I greatly prefer on the whole to use a colloidal solution of copper dissolved in ether.

Of course electrotype molds are ordinarily prepared from wax, but it is well known

that galvano plastic molds are made from other substances also, for instance, gutta percha, plaster of Paris, et cetera. The liquid that I use for a solvent depends upon the composition of the mold. For a mold of gutta percha I employ benzol as a solvent, for I find that a solution prepared from this as a solvent readily wets a gutta percha mold.

10 I find that in practice in using ether as a solvent the operator has to be very rapid in his work on account of the rapidity of evaporation of the ether. Moreover, the ether if too thickly applied makes the wax 15 rather soft. For both of these reasons I sometimes use a mixture of ether and alcohol instead of ether alone.

10 In practicing my method I sometimes pour the colloidal solution onto the mold 20 and thus form a layer upon it or again sometimes apply it with a brush or sometimes dip the mold completely in the colloidal solution.

Having thus described my invention,

what I claim as new, and desire to secure by 25 Letters Patent, is:

1. The herein described process of producing an electrically conductive layer upon the surface of a non-conductive material which consists in first applying to the surface a colloidal solution of a conductive solid in a volatile solvent and then permitting the said solvent to evaporate.

2. The herein described process of producing an electrically conductive layer upon a 35 surface, such as a mold, which consists in first applying to the mold surface a colloidal solution of a metal in a volatile solvent and then permitting the said solvent to evaporate.

40 In witness whereof, I have hereunto subscribed my name in the presence of two witnesses:

HYMAN ELI GOLDBERG.

Witnesses:

HOWARD M. COX,  
MARGARET D. ROBB.